

## UNITED STATES PATENT OFFICE

2,005,488

PROCESS FOR THE PRODUCTION OF  
SILICOFLUORIDES

Emil Gotthilf Leopold Abel, Brand-Erbisdorf, Germany, assignor to Brander Farbwerke, Chemische Fabrik Gesellschaft mit beschränkter Haftung, Brand-Erbisdorf, Germany, a corporation of Germany

No Drawing. Application August 15, 1932, Serial  
No. 628,896. In Germany August 26, 1931

2 Claims. (Cl. 23—88)

The invention relates to a process for the production of silicofluorides,—such, for example, as are used for timber-preserving,—and is particularly adapted to the production of silicofluorides of the metals, as zinc and the like.

5 It is well known, that the salts of silicofluoric acid, particularly the silicofluoride of zinc, are excellent products for preserving wood. But they have a great quantity of acid which is unbound. 10 For that reason they have a destroying effect on metals—especially iron—so that they can not be used for the impregnation of wood in pressure chamber installations, and for that reason they have hitherto played but a subordinate part in the technique of impregnating.

15 As a rule, for example, silicofluoride of zinc is produced by dissolving shavings of zinc in stoicheiometrical relation in silicofluoric acid. Although the process may be very simple, it has nevertheless its difficulties and shows great disadvantages. The complete reaction of the zinc-metal requires an unproportionally long time. In spite of the fact that the metal and the acid do react with each other in equivalent quantities, the process does not react quantitatively. During the reaction of the metal upon the acid, a state of equilibrium arises, so that undissolved zinc and unbound acid remain after the reaction, whereby the solution—or the salt produced by concentration, respectively—becomes useless as a means of impregnating in chamber installations.

20 A further disadvantage of the known processes lies in the fact that the reaction must be carried out in a solution considerably diluted with water, in order to accelerate the process.

25 The invention avoids these disadvantages. It was found that, when producing silicofluorides, extremely pure terminal lye, being absolutely free from acid, is obtained by carrying out the reaction in the presence of a catalyser. Zinc metal, for instance,—particularly in the shape of zinc-dust, reacts upon acid in an extraordinary short time by bringing the equivalent quantity of a metallic catalyser—as, for example, copper reduced and finely precipitated—into the very lazy reaction mixture. The process then becomes quantitative according to the equation:



30 The process in accordance with the invention can, for example, be carried out as follows:

35 The quantity of silicofluoric acid necessary for one charge is brought into the vessel and then 40 the equivalent quantity of reduced copper, in 45

the form of powder, is added. After that the equivalent quantity of zinc dust, which is dry, or mixed with a small quantity of water—in order to avoid the formation of lumps—is added, under stirring. It is stirred until all the zinc-metal has 5 reacted, which can be recognized by the ceasing of the formation of hydrogen-gas. The catalyser, although being metallic and possessing a capacity for reaction, does not react with the silicofluoric acid and can therefore be employed again in the 10 next charge, after having been separated from the solution of silicofluoride of zinc.

15 It is evident that the process, in accordance with the invention, may be varied by supplying the acid first and the zinc-dust afterwards, the 20 mass of catalyzer, which may be in a swelled-up condition, being added last.

25 In view of the complete discussion above with regard to the making of the silicofluoride of zinc, it will be obvious to persons skilled in the art how 20 to make silicofluorides of other metals.

The following experiments may serve to illustrate the technical and economical advantages of the present invention. It may suffice, for the purposes of these experiments, to choose reduced 25 copper as the catalyzer.

## Example No. I—without catalysis

30 There were combined together, under constant stirring, 131 grams of old, scrap zinc, in small chip form, with 348 grams of fluosilicic acid, at 35 degrees Bé (34 per cent). The temperature 35 rose to about 37 degrees C.; and though the reaction was quite intense, at first, it abated rapidly. One and one-half hours later, therefore, 100 40 cubic centimeters of water was added. After twenty hours, the solution was found to have a density of 42 degrees Bé. It was remarkably acid. A further 100 cubic centimeters of water was then 45 added and, after twenty six hours, was again tested, and was found to have a density of 41 degrees Bé. Twenty four hours later, still another 100 cubic centimeters of water was added; after seventy two further hours, it was found, on test, to have a density of 38 degrees Bé. This 45 time, 50 cubic centimeters of water was introduced; and, as no further observable reaction followed, the experiment was terminated, and the resulting composition analyzed. There were 1743 grams of very acid liquor of 26 degrees Bé, 50 containing 556.7 grams  $\text{ZnSiF}_6 + 6\text{H}_2\text{O}$ , counting in the free acid, which also spindles high. This would correspond to a yield of 88.22 per cent. The undissolved zinc metal residue amounted, 55 after drying, to 38.22 per cent of the originally

added metal so that, if the fluosilicic acid not being saturated is subtracted from the above value, there was obtained only a yield of hardly 62 per cent.

5 *Experiment No. II—without catalysis*

This experiment, employing zinc chips, without a catalyst, was repeated, with the only difference that the time of reaction was increased to 10 seven weeks. Since, after the lapse of this time, no further reaction could be observed, the experiment was terminated and the results analyzed. There were found 813 grams of liquor of 28 degrees Bé. (279.67 grams  $ZnSiF_6 \cdot 6H_2O$ ) and 403 15 grams liquor of 0.5 degree Bé. (2.5 grams  $ZnSiF_6 \cdot 6H_2O$ ), or a total of 282.17 grams of  $ZnSiF_6 \cdot 6H_2O$ . This corresponded to 99.42 per 20 cent of the amount that should have been obtained theoretically if the acid being also spindled and not subtracted is included. The liquor was 25 strongly acid. The undissolved zinc residue, when dry, weighed 35.4 grams, which corresponded to 27 per cent of the zinc employed. This consequently gave a yield of 73 per cent.

25 *Experiment No. III—without catalysis*

The same experiment, with the same metal, without the use of a catalyst, was again repeated, but permitting the reaction to take place 30 for only six hours. The results were 774 grams liquor, at 41.5 degrees Bé. and 661 grams liquor, at 14.5 degrees Bé., or a total of 1,435 grams liquor, at 29.5 Bé., corresponding to 520.097 grams  $ZnSiF_6 \cdot 6H_2O$  including the free acid not being 35 saturated.

This product was very strongly acid, and an analytic determination of the end product of the above-mentioned weight showed an acid content of, together, 139.568 grams of the fluo-silicic acid 40 (100 per cent) which, on the other hand, corresponded to 400.47 grams of acid of 35 degrees Bé. It follows that 48.40 per cent of the originally 45 added acid was not utilized; which checks exactly, for the residue of the zinc sheet, well washed and well dried, weighed 64.5 grams, corresponding to 48.48 per cent of the zinc metal originally employed.

The yield, according to this experiment, therefore, was about 51.5 per cent.

50 These three experiments have been carried out with sheet zinc, instead of with zinc dust, in order to demonstrate that the catalytic action of old zinc is quite insufficient for producing a neutral end product. The solution of the metal 55 when the catalyst is employed yields, in a fraction of the time formerly necessary, a nearly quantitative gain without residue, and the end product is fully neutral.

As opposed to this, the experiments based upon 60 the prior-art processes involve an uncommonly long time of reaction and a thoroughly unsatisfactory result, for substantial residues of the metallic zinc are left behind and the end products of the resulting mass are strongly acid, in 65 which condition they are useless.

Two experiments in accordance with the present invention, Nos. IV and V, will now be recounted, the first using scrap zinc, and the other zinc dust; the catalyst used during the reaction, in both cases, as before suggested, being reduced copper.

5 *Experiment No. IV—using the catalyst*

The following are mixed together, while stirring: 131 grams zinc chips, as before, 848 grams fluo-silicic acid, at 35 degrees Bé. (34 per cent), 10 150 grams of the catalyst, moistened with 330 grams water, and 100 grams water as the diluent. After twenty four hours, during which the mixture is frequently stirred, the experiment is 15 ended, and the products analyzed. There results: 671 grams liquor of 44 degrees Bé. (333.54 grams  $ZnSiF_6 \cdot 6H_2O$ ), and 2,400 grams liquor of 10 degrees Bé. (294.864 grams  $ZnSiF_6 \cdot 6H_2O$ ), a total of 628.404 grams, or a gain of 99.58 per cent.

20 The residue of undissolved zinc consists only of traces, and the liquor in which it is contained is fully neutral.

25 *Experiment No. V—using the catalyst*

The same experiment is repeated, but with different proportions and using zinc dust. The following ingredients are employed, in the following proportions: 300 grams zinc dust, 300 30 grams catalyst, 200 grams water for moistening the catalyst, and 2,000 grams fluo-silicic acid, at 35 degrees Bé. The experiment starts at noon, when the temperature of a very strong reaction rises to 85 degrees C., which shows how rapid is the chemical action. Barely half an hour later, 35 the reaction is completed, for the mixture has come fully to rest, and test with Congo red paper shows the solution to be entirely neutral. The total liquor containing also the washing water weighs 5,205 grams with a density of 25 degrees 40 Bé. Analysis of the free acid yields a content of 0.196 per cent in weight of free, one-hundred-per-cent, silico-fluoric acid, which shows that all the added zinc dust has been dissolved. The 45 catalyst, remaining behind and being always ready for repeated use, weighs exactly 300 grams, so that there can not be present any undissolved zinc or any free acid.

55 What I claim is:

1. A process for the production of silico-fluorides out of fluo-silicic acid, particularly for the use of timber preserving, characterized by the fact of carrying out the reaction of fluo-silicic acid upon zinc metal in the presence of reduced copper as catalyst.

2. A process for the production of silico-fluorides out of fluo-silicic acid, particularly for the use of timber preserving, characterized by the fact of carrying out the reaction of fluo-silicic acid upon zinc metal in the presence of reduced copper as catalyst, the copper being present in a quantity equal to the chemical equivalent of the zinc metal.

EMIL GOTTHILF ABEL.